

## UNITED STATES PATENT OFFICE

2,087,803

## LUBRICANT

Bert H. Lincoln and Alfred Henriksen, Ponca City,  
Okla., assignors, by mesne assignments, to The  
Lubri-Zol Development Corporation, Cleveland,  
Ohio, a corporation of Delaware

No Drawing. Application July 27, 1932, Serial No.  
625,190. Renewed January 29, 1937

## 21 Claims.

(CL. 87—9)

Our invention relates to methods for the production of high quality lubricating greases and specifically comprises such products as new compositions of matter.

5 Broadly speaking the art of making and using greases has developed into a specialized field of lubrication. With the rapid advances in the mechanical art over the last few decades it was soon found that straight hydrocarbon oils could 10 not be used under certain special mechanical conditions of high pressures and low speeds where a heavy highly viscous or semi-solid lubricant was required. The grease making art developed to meet these special lubricating requirements 15 and now a very large number of different greases are found on the market. These greases vary in composition over rather wide limits. Some are mixtures of as little as 1% of soap or less, and 99% or more, of relatively light non-viscous hydrocarbon oils, as one extreme and others are mixtures of 60% or more of soap and 40% or less of very heavy viscous hydrocarbons, as the other extreme. A large number of greases varying in composition between these extremes are on the market. The common characteristics of all 20 greases being a mixture of soap and hydrocarbon oil. In addition to these ingredients a large number of other substances are used in greases for various purposes, such as: fillers, odorants or perfume substances, graphite, mica, wax, borax, fibers, rosins, sulfur, etc.—the exact composition of the finished grease depending largely upon the intended use and the ideas of the fabricator and user. Needless to say, the characteristics of the 25 soap and the hydrocarbon oil are also varied for the different greases by varying the alkali or metal and/or the fatty acid or fat.

Up until the present time the grease manufacturer has been able to supply the needs of the machine manufacturer; however, those skilled in the art of manufacturing and using greases are well aware of the fact that many greases are used because they are the best available and 45 not because they preferably meet the requirements of the conditions of use.

The chief objection to greases now available is their relatively low film strength, and the lack of high film strength is probably the primary cause of the failure of the various greases in use

and responsible for lubrication failure and seizure or damaging of the rubbing surfaces.

Since in use greases are subjected to high pressure and slow speeds, their primary object is to give satisfactory lubrication under conditions of boundary lubrication. With boundary lubrication the rubbing surfaces are separated only by a very thin film of lubricant or grease; therefore, the thin film must have very high film strength to give satisfactory lubrication. This is true of all 10 greases irrespective of their exact composition, and to broadly improve greases as a class of lubricants the film strength of the grease must be improved; the various other constituents used in grease manufacture being held constant. 15

Our invention gives the very broad improvement of film strength and is therefore applicable to all greases of all classes, composition and uses.

Objects of our invention are to:

1. Improve the film strength of all lubricant greases.
2. Provide a new type of high pressure grease for all uses.
3. Provide a lubricant grease which will allow 25 the designer of mechanical equipment to design rubbing surfaces of much higher pressure without making changes in mechanical design to overcome changes in physical character of the new greases.

4. Provide greases with substantially the same physical properties as those now in use but with much higher film strength.

5. Cheaply and economically accomplish the above improvements.

In general, our invention consists of halogenation of the fatty acid or fat which is used in preparing the soap, and/or halogenation of the hydrocarbon oil used to blend with the soap, and/or other ingredients in preparation of the 40 finished grease. From this brief statement it is apparent that our invention is applicable to all cup greases, sett greases, soda-base greases, lime base greases, lead base greases, zinc base greases, aluminum base greases, mixed base greases and/or 45 all other grease of whatever name or classification if they contain a soap and hydrocarbon oil.

The halogen may be added to the fatty acid, fat or hydrocarbon oil by any of the known methods. Halogenation by direct addition to the 50

chemically unsaturated molecules followed by chemical substitution and by chemical substitution in the saturated molecules is highly satisfactory. It is not the intention of this invention to cover the method of halogenation, as any of the known methods are satisfactory. The degree of halogenation may be varied over wide limits, depending upon the substance being halogenated and the intended use of the grease containing the halogenated product. The product may be only slightly halogenated and contain as little as one atom of chlorine in each molecule. A higher degree of halogenation is usually used, however, and may be halogenated up to the point of substantially complete halogenation. By the point of "complete halogenation" we mean the point at which the halogenated molecule begins to break down or become unsatisfactory for use, and we do not mean complete hydrogen substitution by halogens.

To prove the efficiency of our invention a grease may be made with the ordinary ingredients in the given proportion with the usual materials. Then another grease may be made in the same manner, with substantially the same proportion of materials but using halogenated fatty acids, fats and/or oils. The two greases thus prepared may be tested on the Timken lubricant tester (a machine developed by the Timken Roller Bearing Company) to determine the film strength of each. It is found that the grease made with the halogenated constituent invariably has the higher film strength. In the Timken lubricant tester the lubricant is used under increasing pressures at the rubbing surface with constant speed until a pressure is reached which causes a breaking down of the grease film and a seizure or damaging of the rubbing surfaces. New rubbing surfaces are used for each test.

To give an example of each grease to which our invention is applicable would only tend to unduly lengthen the specification without making the invention any clearer to those skilled in the art. Examples from a number of classes of greases will be given to show and properly clarify our invention, but are not to be construed as a limitation of the application of the invention.

#### EXAMPLE 1

Stearic acid chlorinated to a melting point of 13° F. and used for making sodium soap after removing excess chlorine.

(a) 2% sodium stearate  
98% of 95 viscosity at 210° F. oil.

(b) 2% sodium soap of chlorinated stearic acid  
98% of 95 viscosity at 210° F. oil.

These two greases tested on Timken machine:

(a) (Straight sodium stearate)—Seizure point at 390 ft./min. 12.9 pound weight, equivalent to approximately 7,800 pounds per square inch.

(b) (Sodium soap of chlorinated stearic acid). seizure point at 390 ft./min. 22.9 pound weight, equivalent to approximately 14,000 pounds per square inch.

From this example it is noted that the film strength of the grease is practically doubled.

#### EXAMPLE 2

A grease prepared similar to that shown in Example 1 but containing 5% of sodium soap of chlorinated stearic acid gave the following tests on the Timken machine:

(a) Straight sodium stearate 2% in 98% of

95 viscosity at 210° F. oil—seizure at a pressure of approximately 7,800 pounds per square inch (see Example 1).

(b) 5% sodium soap of chlorinated stearic acid in 95% of 95 viscosity oil at 210° F.—seizure point at 390 ft./min. 53 pound weight equivalent to approximately 30,000 pounds per square inch.

This example shows more than double the film strength by increasing soap content from 2% to 5%. The film strength of the 5% soap grease made from chlorinated acid is of about 385% higher film strength than the grease containing 2% ordinary sodium stearate.

As the amount of the halogenated soap content is increased in the various greases, the film strength increases as a general rule.

The following examples show some of the possible modifications of our invention by the actual product:

#### EXAMPLE 3

##### TRANSMISSION GREASE (SODA BASE)

|                      | Per cent |
|----------------------|----------|
| Chlorinated tallow   | 2.09     |
| Caustic              | 0.38     |
| 180 pale neutral oil | 7.57     |
| 95@210 F. zero oil   | 89.96    |

#### EXAMPLE 4

##### PRESSURE LUBRICANT (LIME BASE)

|                                   | Per cent |
|-----------------------------------|----------|
| Chlorinated cottonseed fatty acid | 14.43    |
| Lime                              | 2.10     |
| Water                             | 0.36     |
| 300 red oil                       | 80.11    |
| D bright stock                    | 3.00     |

#### EXAMPLE 5

##### #3 CUP GREASE (AUTOMOTIVE) LIME BASE

|                                   | Per cent |
|-----------------------------------|----------|
| Chlorinated cottonseed fatty acid | 19.00    |
| Chlorinated tallow                | 2.12     |
| Lime                              | 2.98     |
| Water                             | 0.71     |
| 150 pale                          | 75.17    |
| Oil of citronella                 | .02      |

By varying the quantities of chlorinated cottonseed fatty acid and chlorinated tallow and lime, the various grades of cup grease can be made.

#### EXAMPLE 6

##### INDUSTRIAL CUP GREASES (LIME BASE)

|                                   | Per cent |
|-----------------------------------|----------|
| Chlorinated cottonseed fatty acid | 14.43    |
| Chlorinated stearic acid          | 5.43     |
| Lime                              | 2.80     |
| Water                             | 0.49     |
| 300 Texas red                     | 66.88    |
| D bright stock                    | 9.97     |

By varying the percentages of various ingredients different grades of grease can be made.

#### EXAMPLE 7

##### ALUMINUM SOAP CUP GREASES

|                                                  | Per cent |
|--------------------------------------------------|----------|
| Aluminum soap made from chlorinated stearic acid | 10.00    |
| 180 pale neutral                                 | 90.00    |

Different consistency greases can be made by varying the percent of aluminum soap.

## EXAMPLE 8

## FIBER GREASES (LIME AND SODA BASE)

## (a) #2 fiber grease (soda base)

|                     | Per cent |
|---------------------|----------|
| Chlorinated tallow  | 13.18    |
| Caustic             | 1.80     |
| Lime                | 0.30     |
| 70 pale neutral oil | 84.72    |

## (b) #3 fiber grease (soda base)

|                                   | Per cent |
|-----------------------------------|----------|
| Chlorinated tallow                | 13.99    |
| Chlorinated cottonseed fatty acid | 2.82     |
| Caustic                           | 2.35     |
| Lime                              | 0.28     |
| 70 pale neutral oil               | 80.56    |

## EXAMPLE 9

## ROCKER ARM LUBRICANT (ALUMINUM BASE)

|                                                  | Per cent |
|--------------------------------------------------|----------|
| Aluminum soap made from chlorinated stearic acid | 10.00    |
| 25 Oleic acid                                    | 0.5      |
| Steam refined cylinder stock                     | 89.5     |

## EXAMPLE 10

## LEAD SOAP TRANSMISSION GREASE (LEAD BASE)

## (a) #1 lead soap transmission grease

|                                                   | Per cent |
|---------------------------------------------------|----------|
| Lead soap made from chlorinated menhaden fish oil | 20.0     |
| 35 Black oil—110@210 viscosity                    | 62.0     |
| 70 pale neutral oil                               | 16.0     |
| Pine tar                                          | 2.0      |

## (b) #2 lead soap transmission grease

|                                                   | Per cent |
|---------------------------------------------------|----------|
| Lead soap made from chlorinated menhaden fish oil | 20.0     |
| Black oil—190@210 viscosity                       | 78.0     |
| Pine tar                                          | 2.0      |

## EXAMPLE 11

## LEAD NAPHTHANATE TRANSMISSION GREASE

|                                                                                     | Per cent |
|-------------------------------------------------------------------------------------|----------|
| Lead soap made from chlorinated naphthenic acids                                    | 20       |
| Black oil (either 110@210 or 190@210 depending on whether for summer or winter use) | 80       |

## EXAMPLE 12

## ALUMINUM SOAP TRANSMISSION GREASE

|                                                  | Per cent                       |
|--------------------------------------------------|--------------------------------|
| Aluminum soap made from chlorinated stearic acid | 4 <sup>3</sup> / <sub>4</sub>  |
| Steam refined stock                              | 95 <sup>1</sup> / <sub>2</sub> |

By varying the aluminum soap made from different halogenated fatty oils and fatty acids, a variety of different consistencies of grease can be made.

## EXAMPLE 13

|                                                  | Per cent |
|--------------------------------------------------|----------|
| Dehydrated soda soap of a halogenated fatty acid | 50       |
| Viscous hydrocarbon oil                          | 50       |

This is a very high quality hard grease used and designated as a "driving journal compound". The relative proportion of halogenated soap and

hydrocarbon oil is subject to variation, depending upon the type of hydrocarbon oil and degree of halogenation, as well as the physical characteristics required in the finished compound.

In each of the above examples, the film strength of the respective greases was greatly increased over like greases made without the halogenation of our invention.

Special equipment is not required for the manufacture of our greases, the usual plant equipment being satisfactory. The oils may be saponified in pressure or atmospheric vessels.

Having thus described our invention, what we claim is:

1. A grease comprising in combination a hydrocarbon oil and a soap of a halogenated higher fatty acid of the aliphatic series.

2. A grease comprising in combination a hydrocarbon oil and a soap of a chlorinated higher fatty acid of the aliphatic series.

3. A grease comprising in combination a hydrocarbon oil and a metal soap of a halogenated higher fatty acid of the aliphatic series.

4. A grease comprising in combination a hydrocarbon oil and a metal soap of a chlorinated higher fatty acid of the aliphatic series.

5. A grease comprising in combination a hydrocarbon oil and a mixture of respective soaps of a plurality of halogenated higher fatty acids of the aliphatic series.

6. A grease comprising in combination a hydrocarbon oil and a mixture of respective soaps of a plurality of chlorinated higher fatty acids of the aliphatic series.

7. A grease comprising in combination a hydrocarbon oil and a soap of a halogenated animal fatty acid.

8. A grease comprising in combination a hydrocarbon oil and a soap of a chlorinated animal fatty acid.

9. A grease comprising in combination a hydrocarbon oil and a soap of halogenated vegetable fatty acid.

10. A grease comprising in combination a hydrocarbon oil and soaps of chlorinated vegetable fatty acids.

11. A grease comprising in combination a hydrocarbon oil and metal soaps of chlorinated vegetable fatty acids.

12. A grease comprising in combination a hydrocarbon oil and a soap of a halogenated fat.

13. A grease comprising in combination a hydrocarbon oil and a soap of a halogenated animal fat.

14. A grease comprising in combination a hydrocarbon oil and a soap of a halogenated vegetable fat.

15. A grease comprising in combination a hydrocarbon oil and a soap of a halogenated fish oil.

16. A grease comprising in combination a hydrocarbon oil, a soap of a halogenated fat and free higher fatty acid of the aliphatic series.

17. A grease comprising in combination a hydrocarbon oil, a soap of a halogenated fat and free halogenated higher fatty acid of the aliphatic series.

18. A grease comprising in combination a hydrocarbon oil, a soap of a halogenated fat and free halogenated higher fatty acid of the aliphatic series.

19. A grease comprising in combination a hydrocarbon oil and a small amount of a soap selected from the following group,—soaps of halogenated higher fatty acids of the aliphatic

series, soaps of halogenated fats, soaps of halogenated oils.

20. A lubricating composition comprising in combination a hydrocarbon oil and about 1% of a soap of a halogenated higher fatty acid of the aliphatic series.

21. A lubricating composition comprising in

combination a hydrocarbon oil and an amount less than 60%, based on the total composition, of a soap of a halogenated higher fatty acid of the aliphatic series.

BERT H. LINCOLN.  
ALFRED HENRIKSEN.